



US005225156A

**United States Patent** [19]

Ototani

[11] **Patent Number:** **5,225,156**[45] **Date of Patent:** **Jul. 6, 1993**[54] **CLEAN STEEL COMPOSITION**

[75] Inventor: Tohei Ototani, Tokyo, Japan

[73] Assignee: Metal Research Corporation, Tokyo,  
Japan[21] Appl. No.: **554,658**[22] Filed: **Jul. 19, 1990**

[56]

**References Cited****U.S. PATENT DOCUMENTS**

|           |         |                |         |
|-----------|---------|----------------|---------|
| 4,054,447 | 10/1977 | Tenmyo .....   | 420/103 |
| 4,091,147 | 5/1978  | Kanazawa ..... | 420/103 |
| 4,318,739 | 3/1982  | Lehman .....   | 420/103 |
| 4,561,888 | 12/1985 | Okuda .....    | 420/103 |
| 4,714,502 | 12/1987 | Honkina .....  | 420/103 |
| 4,946,519 | 8/1990  | Honda .....    | 420/103 |

**Related U.S. Application Data**

[63] Continuation-in-part of Ser. No. 498,069, Mar. 23, 1990, which is a continuation-in-part of Ser. No. 363,570, Jun. 7, 1989, Pat. No. 4,944,798.

[30] **Foreign Application Priority Data**

Feb. 1, 1989 [JP] Japan ..... 1-20817

[51] Int. Cl.<sup>5</sup> ..... C22C 38/28[52] U.S. Cl. ..... **420/103**

[58] Field of Search ..... 420/85, 9, 84, 103,

420/104

*Primary Examiner*—Peter D. Rosenberg*Attorney, Agent, or Firm*—Sughrue, Mion, Zinn, Macpeak & Seas[57] **ABSTRACT**

Disclosed is a clean steel containing less than 30 ppm of oxygen, less than 30 ppm of sulfur, less than 150 ppm of nitrogen, 5 to 0.1 ppm of Mg and 25 to 0.1 ppm of Ca.

**2 Claims, 4 Drawing Sheets**

FIG. 1

Phase diagram of  $\text{CaO}-\text{MgO}$  system

FIG. 2

Phase diagram of  $\text{CaO}-\text{MgO}-\text{Cr}_2\text{O}_3$  system

FIG. 3



FIG. 4

Phase diagram of  $\text{CaO}-\text{MgO}-\text{Al}_2\text{O}_3$  system

FIG. 5



FIG. 6



## CLEAN STEEL COMPOSITION

This application is a continuation-in-part application of U.S. patent application Ser. No. 07/498,069, which is a continuation-in-part application of U.S. patent application Ser. No. 363,570, filed on Jun. 7, 1989 and now U.S. Pat. No. 4,944,798.

## BACKGROUND OF THE INVENTION

## (a) Field of the Invention

The present invention relates to a clean steel made of a ferroalloy of super high purity, and relates to a clean steel containing extremely small amounts of oxygen, sulfur and nitrogen, and small amounts of magnesium and calcium.

## (b) Related Art Statement

The inventor has previously proposed a method of manufacturing molten steel having less contents of oxygen and sulfur as Japanese Patent Laid-open No. 52(1977)-58,010 and Japanese Patent Application Publication No. 62(1987)-37,687.

The inventor has further proposed an iron-, nickel-, and cobalt-base alloy having extremely small contents of sulfur, oxygen and nitrogen and a method of manufacturing the same as Japanese Patent Laid-open No. 62(1987)-83,435.

According to the above prior methods, the residual sulfur is less than 0.002%, the residual oxygen is less than 0.002% and the residual nitrogen is less than 0.03% in the molten steel.

That is, the invention of Japanese Patent Laid-open No. 62(1987)-83,435 relates to a method of manufacturing an iron-base alloy having extremely small contents of oxygen, sulfur and nitrogen comprising a step of substantially melting an iron alloy in a crucible consisting of basic refractories containing 15-75 wt % of MgO and 15-85 wt % of CaO, or a crucible, a crucible melting furnace, a converter or a vessel such as a ladle lined with said refractories, deoxidizing, desulfurizing and denitrifying the molten alloy in a non-oxidizing atmosphere such as argon gas, nitrogen gas or helium gas or in vacuo, by adding first and second additives, the first additive being aluminum or an aluminum alloy, and the second additive being selected from the group consisting of boron, alkali metal and alkali earth metal, and casting the thus deoxidized, desulfurized and denitrified molten alloy into an ingot.

According to this method, in order to remain

|                                                                                                                                |               |
|--------------------------------------------------------------------------------------------------------------------------------|---------------|
| residual Al                                                                                                                    | 0.005-7%      |
| residual Mg                                                                                                                    | 0.005-0.0001% |
| residual Ca                                                                                                                    | 0.005-0.0001% |
| total residual amount of at least one element selected from the group consisting of boron, alkali metal and alkali earth metal | 0.001-10 wt % |

these metals are preferably added.

## SUMMARY OF THE INVENTION

An object of the invention is to improve spalling resistance and hydrating properties as compared with conventional natural dolomite and synthetic calcia-magnesia refractories.

An object of the invention is to provide a clean steel consisting essentially of by weight 0.0001%-0.5% of aluminum, 0.0001%-0.5% of silicon, 0.00001%-0.0005% of magnesium, 0.00001-0.0025%

5 calcium, 0.00001%-0.003% of oxygen, 0.0001%-0.003% of sulfur, and 0.0001%-0.015% of nitrogen, less than 2% of carbon, 0.0001%-0.5% of at least one element selected from the group consisting of titanium, niobium, tantalum and boron and the remainder iron.

10 Another object of the invention is to provide a clean steel consisting essentially of by weight 0.0005%-0.5% of aluminum, 0.0001-0.5% of silicon, 0.00001%-0.0005% of magnesium, 0.00001%-0.0025% of calcium, 0.00001%-0.003% of oxygen, 0.00001%-0.003% of sulfur, and 0.0001%-0.015% of nitrogen, less than 2% of carbon, 0.0001%-0.5% of at least one element selected from the group consisting of titanium, niobium, tantalum and boron, a minor amount 15 of phosphorous and manganese and an alloy steel consisting of 0.001~50% of at least one element selected from the group consisting of nickel, chromium, tungsten, molybdenum, and vanadium and the remainder iron.

20 Another object of the invention is to provide a clean steel consisting essentially of by weight 0.0005%-0.5% of aluminum, 0.0001%-0.5% of silicon, 0.00001%-0.0005% of magnesium, 0.00001%-0.0025% of calcium, 0.00001%-0.003% of oxygen, 0.00001%-0.003% of sulfur and 0.0001%-0.015% of nitrogen, less than 2% carbon and the remainder iron, wherein the clean steel further includes 0.0001%-0.5% of at least one element selected from the group consisting of titanium, niobium, tantalum and boron, wherein 25 said alloy steel further consists of at least one element selected from the group consisting of nickel, chromium, cobalt, tungsten, vanadium and molybdenum as a special alloy steel.

## BRIEF DESCRIPTION OF THE DRAWINGS

30 FIG. 1 is a phase diagram of CaO—MgO refractories used in the present invention;

35 FIG. 2 is a phase diagram of CaO—MgO—Cr<sub>2</sub>O<sub>3</sub> refractories used in the present invention;

40 FIG. 3 is a phase diagram of a ZrO<sub>2</sub>—CaO—MgO composition used in the present invention;

45 FIG. 4 is a phase diagram of CaO—MgO—Al<sub>2</sub>O<sub>3</sub> refractories used in the present invention;

50 FIG. 5 is a phase diagram showing hydration characteristics of CaO, CaO—30%MgO and 20%CrO—CaO—30%MgO in saturated vapor at 50°C.; and

55 FIG. 6 is a graph showing the calcium behavior of the present product in a tundish and a ladle.

## DESCRIPTION OF THE PREFERRED EMBODIMENTS

55 The invention will be explained by referring to the drawings.

FIG. 1 is a phase diagram of CaO—MgO system binary refractories formed by mixing CaO with MgO. FIG. 2 shows a phase diagram of CaO—MgO—Cr<sub>2</sub>O<sub>3</sub>

60 tertiary system refractories. From FIG. 2 of this phase diagram is obtained a mixed structure of CaO—MgO—CaCrO<sub>4</sub> system by adding Cr<sub>2</sub>O<sub>3</sub>. FIG. 3 shows a tertiary phase diagram of refractories of CaO—MgO—ZrO<sub>2</sub>, and as is apparent from FIG. 3, the refractories are a mixed structure of CaZrO<sub>3</sub>+CaO solid solution+MgO.

65 FIG. 4 shows a phase diagram of tertiary refractories of CaO—MgO—Al<sub>2</sub>O<sub>3</sub>, and as is apparent from FIG. 4,

the refractories are a mixed structure of  $\text{CaO}-\text{MgO}-5\text{CaO}3\text{Al}_2\text{O}_3$ . These tertiary refractories apparently contain carbide and silicate in part with respect to quaternary refractories of the present invention which further include C and  $\text{SiO}_2$  in each of these tertiary refractories. 5

The phase diagrams of the refractories according to the present invention are rather complicated depending upon the structure and phase diagram, but there are effects of improving spalling resistance by contents and components of tertiary oxides other than  $\text{CaO}$  and  $\text{MgO}$  as compared with  $\text{CaO}$ ,  $\text{MgO}$  refractories, and more especially, the effect is a remarkably improved, except for quaternary refractories containing silicate. 10

FIG. 5 shows the comparative data of hydration properties by comparing the prior data of the fired refractories with respect to the starting material of  $\text{MgO}-70\%\text{CaO}$  and with the refractories of  $25\%\text{MgO}-56\%\text{CaO}$  containing 18%  $\text{Cr}_2\text{O}_3$ . It becomes clear from these comparative data that hydration resistance is improved by mixing 18% of  $\text{Cr}_2\text{O}_3$ . Hydration properties of refractories made by mixing a tertiary oxide of less than 30% of the present invention with calcia-magnesia ( $\text{CaO}-\text{MgO}$ ) are complicatedly influenced by carbonation and preliminary treatment of the exposed surface, system, porosity and the like, but it is apparent from each phase diagram of the tertiary refractories that a mixed structure is obtained by adding a tertiary oxide, whereby hydration properties are greatly improved. 15

The reducing reaction carried out in the container such as a crucible, a converter or a ladle lined with said refractories of  $\text{CaO}$  of 7-90 wt % and  $\text{MgO}$  of 90-7 wt % which total content is 70-99.9% is as follows.

In each of the above embodiments, a part of aluminum (Al) added as an additive to the molten alloy in the container is directly bonded with oxygen in the molten alloy in vacuo or a non-oxidizing atmosphere so as to generate  $\text{Al}_2\text{O}_3$  for deoxidation, but the other part of aluminum (Al) is reacted with  $\text{MgO}$  and  $\text{CaO}$  in the refractory surface in vacuo or a non-oxidizing atmosphere in accordance with the following equations to generate Mg, Ca and  $\text{Al}_2\text{O}_3$ . 35



The reason why the melting furnace or the container is composed of or lined with refractories having a composition consisting of 90-7% by weight of  $\text{MgO}$  and 7-90% by weight of  $\text{CaO}$  in the present invention will be explained as follows. 50



Calcium aluminate mainly consisting of this  $\text{CaO} \cdot \text{Al}_2\text{O}_3$  has high desulfurizing power, and as a result, the desulfurization of the molten alloy proceeds.

The following reaction also occurs by the presence of titanium (Ti), niobium (Nb), tantalum (Ta) and boron (B) in vacuo or a non-oxidizing atmosphere. 60



In addition to the above reactions, sulfur, oxygen and nitrogen in the molten steel bath are reacted by aluminum (Al), titanium (Ti), niobium (Nb), tantalum (Ta) and boron (B) to be added in the first place as follows.



In addition, the sulfur, oxygen and nitrogen components remaining in the molten bath are removed by magnesium (Mg) and calcium (Ca) reduced and separated in the molten alloy as described above and as shown in the following formulae (25) to (30), and an extremely clean molten steel bath is obtained.

More particularly, the molten steel bath is in vacuo or a non-oxidizing atmosphere and a proper amount of 7-90% of  $\text{CaO}$  and 90-7% of  $\text{MgO}$  is present in the crucible or the lining of container, so that the reaction of the equation (2) easily proceeds on the right side as shown in the formulae (1) and (2). This reaction is considered to be the following complex reaction.



Thus, the deoxidation is carried out by added aluminum (Al), while both the deoxidation and the desulfurization are carried out by the active magnesium (Mg), calcium (Ca) and calcium aluminate ( $3\text{CaO} \cdot \text{Al}_2\text{O}_3$ ) generated by the reducing action of aluminum (Al).

These reactions extremely quickly proceed, and so the desulfurization and deoxidation are almost completed in several minutes after adding aluminum (Al) to the molten steel bath.

Further, the nitrogen content in the molten steel bath is gradually reduced with the lapse of time. This is because nitrogen (N) is separated from the molten steel bath with the evaporation of calcium (Ca), magnesium (Mg) and the like. This denitrifying rate is considerably raised according to the progress of the deoxidation and desulfurization in a non-oxidizing gas or in vacuo or in an atmosphere such as argon gas.

Next, the reason why the components and compositions of refractories are limited in the present invention will be explained as follows.

(a) In the case that the total content of CaO—MgO is 70% to more than 99.9%:

From a refining effect of active Ca and Mg by reducing CaO—MgO of refractories and an effect of improving hydration resistance of a tertiary oxide, the above composition range is determined by taking their harmonic points into consideration.

(b) In the case that  $Al_2O_3$ ,  $Cr_2O_3$ ,  $ZrO_2$ ,  $SiO_2$ ,  $ZrC$  and C are 30—0.1%:

The above composition range is determined by taking the harmonic points for an improved effect of hydration resistance of CaO—MgO and a refining effect of CaO—MgO of refractories by a reducing agent such as Al and the like. (c) In the case of less than 30 ppm of oxygen, less than 30 ppm of sulfur and less than 150 ppm of nitrogen:

As a result of actual operation, the upper limits are determined by aiming at the range for attaining high purity steel.

(d) In the case of 5—0.1 ppm of Mg and 25—0.1 ppm of Ca:

From a result in actual operation, Ca immediately after adding 0.1% of aluminum (Al) becomes 5 to 6 ppm within a tundish, and the calcium (Ca) content of the product becomes 2 to 3 ppm, and hence, the content of residual calcium (Ca) is determined to be less than 25 ppm to 0.1 ppm.

In the same manner, the content of magnesium (Mg) within a tundish is reduced by half in a product, and as a result, the content of residual magnesium (Mg) is determined to be less than 5 ppm to 0.1 ppm.

#### EXAMPLE 1

80% of a CaO—MgO clinker and 20% of a zircon oxide containing 95% of  $ZrO_2$  were mixed and fired at 1,600° C. to manufacture a crucible of 80 mm in outer diameter and about 160 mm in height. A high frequency vacuum induction furnace of 10 kw and 50 KHz was used for melting, and a desired amount of additive metal was added to about 1 kg of an electrolytic iron molten bath, in which the concentration of O and S was previously adjusted, at an argon atmosphere under pressure at 1,600° C.

The additive metal was 0.5% of Al, and at least one element not more than 0.5% and more than 0.001% from Ti, Zr, Ce and the like having a purity of more than 99%, if necessary, is added together with less than 5% of a solvent.

As a result of adding 0.5% of Al, the residual amounts of O, S, N, Mg and Ca in the electrolytic iron molten bath after 10 minutes were O=12 ppm, S=2 ppm, N=27 ppm, Mg=4 ppm, and Ca=1 ppm.

The desulfurization result after an experiment with the use of Ti, Zr and Ce was S=2 ppm after adding Al, and in the case of adding Zr, S=17 ppm, in the case of adding Ti, S=20 ppm, and after adding Ce, S=95 ppm, resulting in less desulfurization effect of rare earth metal.

#### EXAMPLE 2

A Ca—Si alloy was added to an RH vessel, and a Ca—Si clad wire was added to a ladle after completing treatment, in an RH-type cacuum degassing device respectively, and a residual amount of Ca and a morphological change of an inclusion were examined. Table 1 shows the composition of Ca—Si alloy and Ca—Si clad wire added.

TABLE 1

| Material    | Chemical compositions of<br>Ca—Si alloy and Ca—Si wire |      |    |
|-------------|--------------------------------------------------------|------|----|
|             | Fe                                                     | Ca   | Si |
| Ca—Si alloy | —                                                      | 32   | 60 |
| Ca—Si wire  | 55                                                     | 14.4 | 27 |

100 tons of low carbon aluminum killed steel in a ladle was treated in an RH-type vacuum degassing device and continuously cast into a bloom of 250×370 mm. The ladle is lined in a furnace wall with refractory bricks consisting essentially of 56% of CaO, 25% of MgO and 18% of  $Cr_2O_3$ , and as a slag lining, MgO brick was used.

FIG. 6 shows an example of the behavior of Ca. The content of 10-odd ppm of Ca after addition into the ladle became 5—8 ppm in a tundish. Residual Ca was 2-3 ppm and Mg was 3—4 ppm in the product. In the product, O<sub>2</sub>=12—9 ppm, S=8—12 ppm and N<sub>2</sub>=28 ppm. There was no nozzle closure, nor morphological change of the inclusion.

#### EXAMPLE 3

With the use of a ladle of 80 tons having a furnace wall consisting essentially of tertiary refractories of 35% of CaO, 45% of MgO and 18% of  $ZrO_2$ ,  $SiO_2$ , low chromium alloy steel was secondarily refined with basic slag in an RH-type vacuum degassing device.

Into the ladle, 0.1 of a Ca—Si clad wire (55% Fe, 14.4% Ca, 27% Si) was added into the ladle. The analytical result of three typical charges is as shown in Table 2.

TABLE 2

| Sample component | A      | B      | C      |
|------------------|--------|--------|--------|
| C %              | 0.18   | 0.19   | 0.20   |
| Cr %             | 1.15   | 1.27   | 1.10   |
| Ca ppm           | 1.5    | 2.5    | 2.3    |
| Mg ppm           | 1.1    | 1.6    | 1.4    |
| Sol Al %         | 0.035  | 0.038  | 0.039  |
| O <sub>2</sub> % | 0.0010 | 0.0009 | 0.0011 |
| S %              | 0.0018 | 0.0010 | 0.0015 |
| N <sub>2</sub> % | 0.0040 | 0.0035 | 0.0038 |

As described above, both the residual contents of Ca and Mg were less than 5 ppm, but deoxidation and desulfurization effects were as expected.

#### EXAMPLE 4

90% and 95% of a CaO—MgO clinker and 10% and 5% of a zirconium oxide containing 95% of  $ZrO_2$  were

mixed and fired at 1,600° C. to manufacture a crucible of 80 mm in outer diameter and about 160 mm in height.

A high frequency vacuum induction furnace of 10 kw and 50 KHz was used for melting, and a desired amount of additive metal was added to about 1 kg of an electrolytic iron molten bath, in which the concentration of oxygen (O) and sulfur (S) was previously adjusted, in an argon atmosphere under pressure at 1,600° C.

The addition metal was 0.5% of aluminum, and 0.01% by weight of titanium having a purity of more than 99%, if necessary, is added together with less than 5% of a solvent.

As a result of adding 0.5% of aluminum, the residual amounts of oxygen, sulfur, nitrogen, magnesium, titanium and zirconium in the electrolytic iron molten bath after 10 minutes, were as shown in Table 3.

TABLE 3

| Chemical composition of basic refractories |       |       |                    |  |  |  |
|--------------------------------------------|-------|-------|--------------------|--|--|--|
|                                            | CaO % | MgO % | ZrO <sub>2</sub> % |  |  |  |
| First                                      | 47.5  | 47.2  | 5.1                |  |  |  |
| Second                                     | 44.5  | 44.2  | 9.8                |  |  |  |

TABLE 4

| Chemical composition |        |        |        |       |       |        |
|----------------------|--------|--------|--------|-------|-------|--------|
| O <sub>2</sub> %     | S %    | N %    | Ti %   | Zr %  | Ca %  | Mg %   |
| First                | 0.0001 | 0.0001 | 0.0010 | 0.008 | 0.004 | 0.0002 |
| Second               | 0.0003 | 0.0001 | 0.0008 | 0.007 | 0.021 | 0.0003 |

5% and 10% of ZrO<sub>2</sub> and a CaO—MgO clinker containing 50% CaO and 50% of MgO were mixed and

fired at 1,600° C. to manufacture a crucible in the same manner as in Example 1. As a result, it was found that the refining effect is substantially the same even by changing ZrO<sub>2</sub> between 5 to 10%, and that there is no great difference. Therefore, it becomes clear that a refractory material consisting of a mixture of a CaO—MgO refractory material and ZrO<sub>2</sub> is effective in economy, resistance against hydration, and spalling.

What is claimed is:

1. A clean steel consisting essentially of by weight 0.0001%—0.5% of aluminum, 0.0001%—0.5% of silicon, 0.00001%—0.0005% of magnesium, 0.00001—0.0025% of calcium, 0.00001%—0.003% of oxygen, 0.0001%—0.003% of sulfur, and 0.0001%—0.015% of nitrogen, less than 2% of carbon, 0.0001%—0.5% of at least one element selected from the group consisting of titanium, niobium, tantalum and boron and the remainder iron.

2. A clean steel consisting essentially of by weight 0.0005%—0.5% of aluminum, 0.0001%—0.5% of silicon, 0.00001%—0.0005% of magnesium, 0.00001%—0.0025% of calcium, 0.00001%—0.003% of oxygen, 0.00001%—0.003% of sulfur and 0.0001%—0.015% of nitrogen less than 2% carbon and the remainder iron, wherein the clean steel further include 0.0001%—0.5% of at least one element selected from the group consisting of titanium, niobium, tantalum and boron, wherein said alloy steel further consists of at least one element selected from the group consisting of nickel, chromium, cobalt, tungsten, vanadium and molybdenum as a special alloy steel.

\* \* \* \* \*